

# United States Patent Office

2,859,147

Patented Nov. 4, 1958

1

2,859,147

## PROCESS OF AND COMPOSITIONS FOR PRODUCING COATED ALUMINUM AND ALUMINUM ALLOYS

Bruno R. Jeremias, Chicago, Ill., assignor to Poor & Company, Chicago, Ill., a corporation of Delaware

No Drawing. Application August 27, 1954  
Serial No. 452,700

14 Claims. (Cl. 148—6.16)

This invention relates to a process of and compositions for producing coated aluminum and aluminum alloys in which the coating is colorless to a distinctive blue to bluish green color, and provides excellent corrosion resistance as such or as a paint base.

One of the objects of the invention is to provide a new and improved process for forming a coating on aluminum and aluminum alloys which is highly resistant to corrosion.

Another object is to provide a new and improved process for forming a distinctive blue to bluish green coating on aluminum and aluminum alloys.

Still a further object is to provide a new and improved process for applying a coating to aluminum and aluminum alloys which adheres to such alloys and also provides an excellent paint base to which paints and other organic finishes may be applied.

Another object of the invention is to provide a process for forming such a coating on aluminum and aluminum alloys in a relatively simple and inexpensive manner.

Still a further object is to produce new and improved coating compositions which, when applied to aluminum or aluminum alloys, form a film or coating on the surface thereof, providing excellent corrosion protection.

An additional object of the invention is to provide new and improved corrosion resistant articles made from aluminum and aluminum alloys. Other objects will appear hereinafter.

These objects are accomplished in accordance with the invention by applying to aluminum and aluminum alloys an aqueous solution consisting essentially of chromic acid, phosphoric acid, a complex salt of acetic acid containing combined but undissociated acetic acid, and fluoroboric acid, dissolved in water, with or without a chloride of a metal (including also ammonium) which dissolves in the solution and does not form insoluble precipitates with the other ingredients of the solution. The coating solution which is applied to the aluminum or aluminum alloy is heated preferably until a blue to blue-green color develops. The preferred procedure is to immerse the surface of the aluminum or aluminum alloy in a bath containing the solution which is heated to the desired temperature. The time of heating will depend upon the temperature used and the amount of protection desired. A period of heating of one minute at a temperature of about 120° F. provides substantial corrosion protection but normally produces no substantial color formation on the coated article. A period of fifteen minutes of heating at a temperature of 140° F. is generally sufficient to develop a blue-green color. At higher temperatures of, say 180°—190° F., the blue-green color can be developed in a shorter period of time, say, three to five minutes. At temperatures as low as 80° F. no substantial protective coating is provided.

After the aluminum or aluminum alloy article has been coated the presence of the protective coating can be determined by boiling in water for fifteen minutes. If there is no protective coating, the article will normally

2

turn dark. The blue to blue-green coatings, on the other hand, are not substantially affected by the boiling tests.

In the practice of the invention, it is preferable to prepare the chromic acid in one solution and the fluoroboric acid in a separate solution. The phosphoric acid and the complex salt of acetic acid containing combined but undissociated acetic acid is preferably included in the first solution. The soluble chloride, if one is used, is preferably included in the second solution. Examples of such solutions are:

| Ingredients                                        | Proportions,<br>grams per<br>liter |
|----------------------------------------------------|------------------------------------|
| Composition A:                                     |                                    |
| CrO <sub>3</sub> .....                             | 200                                |
| H <sub>3</sub> PO <sub>4</sub> (75% solution)..... | 315                                |
| Sodium diacetate.....                              | 100                                |
| Water sufficient to make a liter of solution.      |                                    |
| Composition B:                                     |                                    |
| HBF <sub>4</sub> (47% solution in water).....      | 330                                |
| NH <sub>4</sub> Cl.....                            | 7.5                                |
| Water sufficient to make a liter of solution.      |                                    |

An alternative fluoroboric acid solution has the following composition:

| Ingredients                                   | Proportions,<br>grams per<br>liter |
|-----------------------------------------------|------------------------------------|
| Composition B':                               |                                    |
| HBF <sub>4</sub> (47% solution in water)..... | 270                                |
| NH <sub>4</sub> Cl.....                       | 60                                 |
| Water sufficient to make a liter of solution. |                                    |

The above-described solutions may be considered as concentrates suitable for use in preparing the solutions that are actually employed in coating the aluminum or aluminum alloys. Compositions A and B (or B') are separately prepared because if they are mixed together in their concentrated form precipitation of an insoluble substance of unknown composition occurs.

The final composition for coating the aluminum or aluminum alloy is prepared by adding composition A and composition B to a large volume of water. For example, a preferred final composition consists of approximately 2% by volume of composition A and 2% by volume of composition B dissolved in water and a preferred practice is to immerse the aluminum or aluminum alloy surfaced article in this solution at 150° F. for 5 to 20 minutes.

The preferred coating solution contains 4 grams of CrO<sub>3</sub>, 6.3 grams of H<sub>3</sub>PO<sub>4</sub> (75% by weight), 2 grams of sodium diacetate, and 2.68 grams of HBF<sub>4</sub> expressed as F (fluorine), dissolved in sufficient water to form a liter of solution. The optimum weight ratio of F to CrO<sub>3</sub> is 0.7. The range of F to CrO<sub>3</sub> in the coating solution can vary from 0.44 to about 2.2.

The pH of the coating solution is preferably within the range of 1 to 2, and the preferred pH range is from 1.15 to 1.55. A pH as low as .88 is unsatisfactory.

The invention will be illustrated but is not limited by the following examples in which the quantities are stated in parts by weight unless otherwise indicated.

### Example 1

A coating solution is prepared by dissolving 1% by volume of composition A and 1% by volume of composition B' in water. The weight ratio of F to CrO<sub>3</sub> in this composition is approximately .55. The weight ratio of phosphorus as PO<sub>4</sub> to F in this composition is approximately 2.08. The weight ratio of CrO<sub>3</sub> to F is about 1.82.

## Example 2

A coating solution is prepared by dissolving 5% by volume of composition A and 4% by volume of composition B' in water. The weight ratio of F to  $\text{CrO}_3$  is about .44. In this coating solution the weight ratio of  $\text{CrO}_3$  to F is approximately 2.27.

## Example 3

A coating solution is prepared by dissolving 1% by volume of composition A and 4% by volume of composition B' in water. The weight ratio of F to  $\text{CrO}_3$  in this composition is about 2.2.

## Example 4

A coating solution is prepared by dissolving 1% by volume of composition A and .2% by volume of composition B' in water. The weight ratio of F to  $\text{CrO}_3$  in this composition is about 1.1. In this coating solution the weight ratio of phosphorus as  $\text{PO}_4$  to F is approximately 1.04. The weight ratio of  $\text{CrO}_3$  to F is approximately 0.9.

## Example 5

A coating solution is prepared by dissolving 1% by volume of composition A and 1% by volume of composition B' in water. The weight ratio of F to  $\text{CrO}_3$  in this composition is approximately .7. The weight ratio of  $\text{CrO}_3$  to F is approximately 1.43.

## Example 6

A coating solution is prepared by dissolving 1% by volume of composition A and 2% by volume of composition B' in water. The weight ratio of F to  $\text{CrO}_3$  in this composition is approximately 1.4. The weight ratio of  $\text{CrO}_3$  to F is approximately .715.

## Example 7

A coating solution is prepared by dissolving 5% by volume of composition A and 4% by volume of composition B' in water. The weight ratio of F to  $\text{CrO}_3$  is approximately .55. The weight ratio of  $\text{CrO}_3$  to F is approximately 1.78.

## Example 8

A coating solution is prepared by dissolving 2% by volume of composition A and 2% by volume of composition B' in water. The pH of the resultant composition is approximately 1.5.

## Example 9

Each of the solutions described in Examples 1 to 8 is applied as a coating to wrought aluminum alloys 2S, 3S, 24S, 61S and 75S, respectively, by immersing a plate or other article formed from such alloys in each of the coating solutions for periods of time from 1 to 20 minutes at temperatures of from 120° to 150° F.

At a temperature of 120° F. in an immersion time of 1 minute in a coating solution of Example 8, a bright transparent colorless corrosion-resistant coating was obtained.

In the coating solution of Example 8 an excellent blue to blue-green color is developed at a temperature of 150° F. in an immersion time from 5 to 20 minutes. In general, the higher the temperature and the longer the time of immersion, the deeper the color. While it is possible with some alloys to carry out the process at temperatures up to the boiling point of the solution, with other alloys, such as 24S, it is desirable to operate at temperatures around 150° F.

## Example 10

In the coating solution of Example 1 at a temperature of 180°-190° F. a very light blue-green color was developed on aluminum and aluminum alloys in about 5 minutes.

## Example 11

In the coating solution of Example 3 a deeper color than that developed with the coating solution of Example 1 was formed at 180°-190° F. in about 5 minutes.

In this coating solution a light color was formed on aluminum and aluminum alloys at 180°-190° F. in one minute.

In practicing the invention, the chromium contained in the coating solution is used up during the process, and the fluoroboric acid is removed to some extent from the coating solution by dragout. The chromium content is maintained by adding additional quantities of composition A, and the fluoroboric acid content is maintained by adding additional quantities of composition B or composition B'. The pH is also maintained by the addition of compositions A and B (or B').

After the aluminum and aluminum alloy articles are removed from the coating solution they are rinsed with water which may be cold and is preferably not heated to temperatures higher than 140° F.

Generally speaking, the optimum operating conditions involve the use of a temperature of the coating solution of 150° F., a pH of about 1.35 and an immersion time of 10 to 20 minutes or longer, if necessary, until the desired color is obtained, but ordinarily the immersion time should not exceed 30 minutes because the coating is not adherent. Even 30 minutes is too long with some alloys.

30 The complex salts of acetic acid containing combined but undissociated acetic acid are derived by replacing one or more molecules of water in sodium acetate with a molecule of undissociated acetic acid and are well known chemicals. Examples of such substances are the calcium, sodium and potassium salts. However, sodium diacetate

35 is the principal salt of this type available commercially. The function of the complex water soluble salt of acetic acid containing combined but undissociated acetic acid is not clearly understood but it serves in some way to permit the aluminum or aluminum alloy to be immersed in the chromic acid solution for a longer period of time than would be otherwise possible and still obtain a satisfactory product. This in turn makes it possible to obtain the optimum deposition of chromium and a deep blue color without destroying the adherence of the chromium film to the aluminum or aluminum alloy. The quantity of complex acetate in the coating solution, calculated as sodium diacetate, is preferably 0.1 to 5.0 grams per liter. Larger amounts which do not cause discoloration can be employed but serve no useful purpose.

40 The employment of the ammonium chloride or other chloride, such as sodium chloride or potassium chloride, is optional and the quantity used may be varied. In general, however, the quantity of ammonium chloride based on the total weight of  $\text{HBF}_4$  and  $\text{NH}_4\text{Cl}$  is within the range of 4% to 32% by weight. The employment of the chloride apparently results in the formation of a stronger film on the aluminum or aluminum alloy.

45 The weight ratio of phosphorus as  $\text{PO}_4$  to F in the coating solution is preferably within the range of about 1:2 to 4.5:1.

50 The invention provides a new and improved process for obtaining protection against corrosion on aluminum and aluminum alloys. It also provides a process for producing strongly adherent blue to blue-green colored corrosion-resistant films on aluminum and aluminum alloys. Additionally it provides a process of forming films on aluminum and aluminum alloys which are resistant to corrosion and are receptive to paints and other organic finishes.

55 The term "aluminum alloy" as used herein refers to alloys of aluminum and other metals in which aluminum forms the major proportion by weight of the alloy.

Such alloys are well known in the art and include casting alloys as well as wrought alloys. Wrought aluminum alloy 2S contains a minimum of 99% by weight of aluminum. Alloy 3S contains approximately 1.2% by weight manganese, the remainder being aluminum. Alloy 24S contains 4.5% by weight copper, 0.6% by weight manganese, 1.5% by weight magnesium, and the remainder aluminum. Alloy 61S contains 0.6% by weight silicon, 0.25% by weight copper, 1.0% by weight magnesium and 0.25% by weight chromium, the remainder being aluminum. Alloy 75S contains 1.6% by weight copper, 2.5% by weight magnesium, 0.3% by weight chromium and 5.6% by weight zinc, the remainder being aluminum. Of the casting alloys, casting alloy No. 13 contains about 12.0% by weight silicon, the remainder being aluminum. Casting alloy No. 43 contains 5.0% by weight silicon, the remainder being aluminum. Casting alloy No. 85 contains 4.0% by weight copper and 5.0% by weight silicon, the remainder being aluminum.

The expressions "aluminum surfaced article" and "aluminum alloy surfaced article" are intended to include and cover articles in which at least the surface of the article is composed of aluminum and aluminum alloys respectively.

The invention is hereby claimed as follows:

1. A process of applying a protective coating to aluminum and aluminum alloys which comprises applying to aluminum and aluminum alloys with heating to a temperature above about 120° F. an aqueous solution consisting essentially of chromic acid, phosphoric acid, a complex water soluble salt of acetic acid containing combined but undissociated acetic acid derived by replacing water in an acetate salt with acetic acid, and fluoboric acid dissolved in water, the weight ratio of F to  $\text{CrO}_3$  in the coating solution being within the range from 0.44 to about 2.2, the quantity of said complex salt being at least 0.1 gram per liter of solution, and the pH of the coating solution being within the range from about 1 to about 2 until a protective coating is formed.

2. A process of applying a protective coating to aluminum and aluminum alloys which comprises applying to aluminum and aluminum alloys with heating to a temperature above about 120° F. an aqueous solution consisting essentially of chromic acid, phosphoric acid, a complex water soluble salt of acetic acid containing combined but undissociated acetic acid derived by replacing water in an acetate salt with acetic acid, and fluoboric acid dissolved in water, the weight ratio of F to  $\text{CrO}_3$  in the coating solution being approximately 0.7, the quantity of said complex salt being at least 0.1 gram per liter of solution, and the pH of the coating solution being within the range from about 1.15 to about 1.55 until a protective coating is formed.

3. A process of applying a protective coating to aluminum and aluminum alloys which comprises applying to aluminum and aluminum alloys with heating to a temperature above about 120° F. an aqueous solution consisting essentially of chromic acid, phosphoric acid, a complex water soluble salt of acetic acid containing combined but undissociated acetic acid derived by replacing water in an acetate salt with acetic acid, and fluoboric acid dissolved in water, the weight ratio of F to  $\text{CrO}_3$  in the coating solution being within the range from 0.44 to about 2.2, the quantity of said complex salt being at least 0.1 gram per liter of solution, and the pH of the coating solution being within the range from about 1 to about 2 until a blue to blue-green coating is formed.

4. A process of producing an aluminum alloy containing a blue to blue-green coating which is adherent and resistant to corrosion comprising immersing the surface of the aluminum alloy in an aqueous acetic solution consisting essentially of chromic acid, phosphoric

acid, sodium diacetate and fluoboric acid dissolved in water, the weight ratio of F to  $\text{CrO}_3$  in the resultant solution being within the range from 0.44 to about 2.2, the quantity of sodium diacetate being within the range of 0.1 to 5 grams per liter of solution, the pH of said solution being within the range from 1.15 to 1.55, the temperature of said solution being within the range from 120° F. to about 150° F. for a period of time from 5 to 20 minutes.

5. A process as claimed in claim 4 in which said solution contains 4% to 32% by weight, calculated as  $\text{NH}_4\text{Cl}$ , of a water soluble ionizable chloride which does not form insoluble precipitates with the other ingredients of the solution.

6. A process as claimed in claim 5 in which said chloride is ammonium chloride.

7. A coating composition for aluminum and aluminum alloys consisting essentially of chromic acid, phosphorus acid, a complex water soluble salt of acetic acid containing combined but undissociated acetic acid derived by replacing water in an acetate salt with acetic acid, and fluoboric acid dissolved in water, the weight ratio of F to  $\text{CrO}_3$  being within the range from 0.44 to about 2.2, the quantity of said complex salt being at least 0.1 gram per liter of solution, and the pH being within the range from 1 to 2.

8. A coating composition for aluminum and aluminum alloys consisting essentially of chromic acid, phosphoric acid, a complex water soluble salt of acetic acid containing combined but undissociated acetic acid derived by replacing water in an acetate salt with acetic acid, and fluoboric acid dissolved in water, the weight ratio of F to  $\text{CrO}_3$  being about 0.7, the quantity of said complex salt being at least 0.1 gram per liter of solution, and the pH being within the range from 1.15 to 1.55.

9. A coating composition for aluminum and aluminum alloys consisting essentially of chromic acid, phosphoric acid, sodium diacetate and fluoboric acid dissolved in water, the weight ratio of F to  $\text{CrO}_3$  being within the range from 0.44 to about 2.2, the quantity of sodium diacetate being within the range of 0.1 to 5 grams per liter of solution, and the pH being within the range from 1 to 2.

10. A coating composition for aluminum and aluminum alloys consisting essentially of chromic acid, phosphoric acid, sodium diacetate and fluoboric acid dissolved in water, the weight ratio of F to  $\text{CrO}_3$  being within the range from 0.44 to about 2.2, the quantity of sodium diacetate being within the range of 0.1 to 5 grams per liter of solution, and the pH being within the range from 1.15 to 1.55.

11. A coating composition consisting essentially of chromic acid, phosphoric acid, sodium diacetate and fluoboric acid dissolved in water in the approximate proportions of 4 grams of  $\text{CrO}_3$ , 6.3 grams of 75% by weight aqueous  $\text{H}_3\text{PO}_4$ , 2 grams of sodium diacetate, and 2.68 grams of  $\text{HBF}_4$ , calculated as F, per liter of solution.

12. A coating composition for aluminum and aluminum alloys consisting essentially of chromic acid, phosphoric acid, sodium diacetate, fluoboric acid and ammonium chloride dissolved in water, the weight ratio of F to  $\text{CrO}_3$  being within the range from 0.44 to about 2.2, the pH being within the range from 1.15 to 1.55, the weight ratio of phosphorus as  $\text{PO}_4$  to F being within the range from about 1:2 to about 4.5:1, the quantity of sodium diacetate being within the range from about 1 gram per liter to about 5 grams per liter and the quantity of ammonium chloride based on the total weight of  $\text{HBF}_4$  and  $\text{NH}_4\text{Cl}$  being within the range of 4% to 32% by weight.

13. Aluminum and aluminum alloys containing a blue to blue green protective coating produced by the process of claim 1.

14. An aluminum alloy containing a blue to blue green protective coating produced by the process of claim 1.

## References Cited in the file of this patent

5

## UNITED STATES PATENTS

2,438,877 Spruance Mar. 30, 1948

2,459,365 Coates Jan. 18, 1949  
2,507,956 Bruno et al. May 16, 1950  
2,678,291 Spruance et al. May 11, 1954

## FOREIGN PATENTS

259,454 Switzerland Jan. 31, 1949  
54,075 Netherlands Oct. 15, 1942